# EUROPEAN PATENT SPECIFICATION

(11) **EP 2 221 391 B1**
(45) Date of publication and mention of the grant of the patent: **30.04.2014**
(21) Application number: 08847798.9
(22) Date of filing: 05.11.2008
(51) Int. Cl.: C22C 9/06, B21B 3/00, C22C 9/04, C22F 1/08, C22F 1/00

(54) **COPPER ALLOY SHEET**
KUPFERLEGIERUNGSBLECH
FEUILLE EN ALLIAGE DE CUIVRE

(30) Priority: 05.11.2007 JP 2007287066
(43) Date of publication of application: 25.08.2010
(73) Proprietor: The Furukawa Electric Co., Ltd., Chiyoda-ku Tokyo 100-8322 (JP)
(72) Inventor: KANEKO, Hiroshi, Tokyo 100-8322 (JP); HIROSE, Kiyoshige, Tokyo 100-8322 (JP); MIHARA, Kuniteru, Tokyo 100-8322 (JP); EGUCHI, Tatsuhiko, Tokyo 100-8322 (JP)
(74) Representative: Forstmeyer, Dietmar
(86) International application number: PCT/JP2008/070139
(87) International publication number: WO 2009/060873

(56) References cited:
- EP-A1- 0 949 343
- EP-A1- 1 873 266
- JP-A- 3 236 432
- JP-A- 5 156 392
- JP-A- 2002 180 165
- JP-A- 2002 266 042
- JP-A- 2006 152 392
- JP-A- 2006 161 148
- JP-A- 2006 265 731
- JP-A- 2006 265 731
- JP-A- 2006 283 059
- JP-A- 2007 231 364
- US-A1- 2005 236 074
- US-A1- 2005 263 218
- US-A1- 2007 131 315

## Description

### Technical Field

The present invention relates to a copper alloy sheet

### Background Art

Characteristics that are required for copper alloy sheet material that is used for electrical / electronic equipment include for example, constant electrical conductivity, constant tensile strength, constant bending workability, and constant stress relaxation resistance. In recent years, as electrical / electronic equipment have become more compact, more lightweight, more highly functional and more densely packaged, and as the operating temperature has increased, the level of these required characteristics has also increased.

Conventionally, in addition to iron-based materials, copper-based materials such as phosphor bronze, red brass and brass have typically been used as materials for electrical / electronic equipment. Through a combination of solid solution strengthening using Sn or Zn, and work hardening by cold working such as rolling or drawing, the strength of these alloys has been improved. However, alloys that are obtained through these strengthening methods have insufficient electrical conductivity for the recent required level, and since high strength is obtained by adding a high cold working rate, the bending workability and stress relaxation resistance are also insufficient.

As an alternative strengthening method, precipitation strengthening causes microscopic secondary-phase particles on a nanometer order to precipitate into a material. In addition to increasing strength, this strengthening method has the merit of simultaneously improving the electrical conductivity, so it is used in many alloy systems. Of these, Cu-Ni-Si system alloys that are strengthened by precipitating microscopic Ni and Si compounds into Cu (for example, CDA70250, which is a registered alloy of the CDA (Copper Development Association); refer to patent documents 1 and 2) are increasingly being used in the market.

Patent document 1: JP-A-1999-43731
Patent document 2: JP-T-2005-532477

JP 2006 265731 discloses another copper alloy suitable for a connector and a terminal for electric or electronic equipment. US 2005/0263218 A1 discloses another copper alloy for electronic machinery and tools.

-US 2005/0236074 A1 discloses another copper alloy. JP 2007 231364 discloses another copper alloy sheet material and its production method.

### Disclosure of the Invention

Generally, in the case of precipitation-hardened alloys, before aging precipitation heat treatment for obtaining a microscopic precipitation state, solution heat treatment is employed as an intermediate process for solidifying the solution of solute atoms. The temperature of this process differs depending on the alloy system and the solute concentration, however, is a high temperature of about 750 °C. Since the temperature of this solution heat treatment is a high temperature, there is a problem in that the grain size of the material becomes coarse. When the grain size is coarse, problems occur such as cracking due to the promotion of localized deformation during bending, concentration of electric current when bent sections are used as contacts due to large creases on the surface of the bent sections, or cracking of plating that is coated on the surface of the material. Moreover, when the temperature of the solution heat treatment is lowered in order to prevent the grain size from becoming coarse, problems occur in that the amount of atoms that enter into solid solution decreases, the density of microscopic precipitate in the aging treatment decreases, the amount of age hardening decreases and the material strength decreases.

Therefore in solution heat treatment at a temperature at which solute Ni and Si atoms can sufficiently enter into solid solution, there is a demand for technology by which the grain size can be kept small and material having high strength and good bending workability can be obtained.

Taking the aforementioned problems into consideration, it is the object of the present invention to provide a copper alloy sheet material for use in electrical / electronic equipment that has excellent bending workability and strength.

The inventors performed research of copper alloys suitable for use in electrical / electronic equipment, and by focusing their attention on methods of dispersing second-phase particles in order to greatly improve the bending workability and strength of Cu-Ni-Si series copper alloys, developed the present invention after much dedicated study. In addition, the inventors found the best modes of the present invention by discovering added elements that function to improve the strength and stress relaxation resistance characteristics without impairing electrical conductivity. The second-phase particles referred to here are precipitates and crystallized matter.

The following means being claimed are provided with the present invention:
(1) A copper alloy sheet having a tensile strength of 730 to 820 MPa, and consisting of:
   1.8 to 3.3 mass% of Ni,
   0.4 to 1.1 mass% of Si,
   0.01 to 0.5 mass% of Cr,
   optionally 0.01 to 1 mass% in total of at least one element selected from Sn, Mg, Ag, Mn, Ti, Fe and P,
   optionally 0.01 to 1.0 mass% of Zn, and
   optionally 0.01 to 1.5 mass% of Co,
   with the balance being Cu and inevitable impurities;
      wherein when the sheet width and the sheet thickness at the time where the copper alloy sheet is bent by 180° tight bending, the bending work being performed according to JIS Z2248, without causing any cracks are taken to be W, in a unit of mm, and T, in a unit of mm, the product of W and T, in a unit of mm², is 0.16 or less;
      wherein second-phase particles existing on a grain boundary exist at a density of 10⁴ to 10⁸ particles/mm², and the average grain size is 10 µm or less; and
      wherein the copper alloy sheet is obtainable by a method comprising the steps of:
   casting at a cooling rate of 0.1 to 100°C/sec;
   heat treatment or homogenization heat treatment at 900 to 1050°C for 0.5 to 10 hours;
   hot working at a reduction percentage of 50% or greater, and a processing temperature of 600°C or greater, followed by rapid cooling at a cooling rate of 10°C/sec or greater;
   cold working (1) with a reduction percentage of 90% or greater;
   solution heat treatment at 720 to 860°C for 3 sec to 2 hours, wherein during the rise of temperature from 400°C to 700°C, a rate of temperature rise is 0.1°C/sec to 200°C/sec;
   cold working (2) with a reduction percentage of 5 to 50%; heat treatment or aging precipitation heat treatment at 400°C to 540°C for 5 min to 10 hours,
   cold working (3) with a reduction percentage of greater than 0% but not exceeding 10%, and
   annealing or strain relief annealing at 200°C to 600°C for 15 sec to 10 hours.
(2) A copper alloy sheet having a tensile strength of 730 to 820 MPa, and consisting of:
   1.8 to 3.3 mass% of Ni,
   0.4 to 1.1 mass% of Si,
   0.01 to 0.5 mass% of Cr,
   optionally 0.01 to 1 mass% in total of at least one element selected from Sn, Mg, Ag, Mn, Ti, Fe and P,
   optionally 0.01 to 1.0 mass% of Zn, and
   optionally 0.01 to 1.5 mass% of Co,
   with the balance being Cu and inevitable impurities; wherein when the sheet width and the sheet thickness at the time where the copper alloy sheet is bent by 180° tight bending, the bending work being performed according to JIS Z2248, without causing any cracks are taken to be W, in a unit of mm, and T, in a unit of mm, the product of W and T, in a unit of mm², is 0.16 or less;
   wherein the value of ratio r/f of the particle size r, in a unit of µm, of second-phase particles inside the grain and on the grain boundary and the volume fraction f, in a unit of vol.%, of the particles is at least 1 and not more than 100 µm/vol.%, and the average grain size is 10 µm or less; and wherein the copper alloy sheet is obtainable by a method comprising the steps of:
   casting at a cooling rate of 0.1 to 100°C/sec;
   heat treatment or homogenization heat treatment at 900 to 1050°C for 0.5 to 10 hours;
   hot working at a reduction percentage of 50% or greater, and a processing temperature of 600°C or greater, followed by rapid cooling at a cooling rate of 10°C/sec or greater;
   cold working (1) with a reduction percentage of 90% or greater;
   solution heat treatment at 720 to 860°C for 3 sec to 2 hours, wherein during the rise of temperature from 400°C to 700°C, a rate of temperature rise is 0.1°C/sec to 200°C/sec;
   cold working (2) with a reduction percentage of 5 to 50%;
   heat treatment or aging precipitation heat treatment at 400°C to 540°C for 5 min to 10 hours,
   cold working (3) with a reduction percentage of greater than 0% but not exceeding 10%, and
   annealing or strain relief annealing at 200°C to 600°C for 15 sec to 10 hours.
(3) The copper alloy sheet of item (1) or item (2) wherein of the second-phase particles, the ratio of particles comprising Cr as a constituent element is 50% or more.
(4) The copper alloy sheet of any one of the items 1 to 7 wherein, when the copper alloy sheet is maintained at 165 °C for 3000 hours, the stress relaxation rate is 30% or less.

The above and other features and advantages of the present invention will become better understood from the following detailed description with reference to the accompanying drawings.

### Brief Description of the Drawings

FIG. 1 is a drawing explaining a method for testing stress relaxation resistance, where (a) of FIG. 1 shows before heat treatment and (b) of FIG. 1 shows after heat treatment.
FIG. 2 is a graph showing the results of whether or not cracking occurs when the sheet width W (mm) and sheet thickness T (mm) of a test specimen are varied in examples and comparative examples.

### Best Mode for Carrying Out the Invention

The preferred embodiment of the copper alloy sheet of the present invention is explained in detail.

The tensile strength of the copper alloy sheet of the present invention is 730 to 820 MPa. More preferably, it is 740 to 800 MPa. The bending workability is such that under rigid conditions such as when the product of the material sheet width W (mm) and the material sheet thickness T (mm) is 0.16 (mm²) or less, 180° tight bending is possible. It is preferred that this product of width W and thickness T be 0.14 or less. The minimum value of this product of width W and thickness T is not especially limited, however is normally 0.01 or greater.

Moreover, an electrical conductivity of 30% IACS is preferred, and it is also preferred for the stress relaxation resistance that when the material is maintained for 3000 hours or more at 165 °C, the stress relaxation rate be 30% or less.

Suitable dispersion of second-phase particles is effective against grain coarsening during solutionization that causes bending workability to worsen. This is because it is considered that when grain is grown, a gain in energy occurs at the interface between the dispersed particles and grain boundary when the grain boundary passes the second-phase particles and suppresses grain boundary migration.

The obtained grain size is 10 µm or less, and preferably 8 µm or less, and more preferably 6 µm or less. The minimum value of grain size is not particularly limited, however, normally is 2 µm or more. The grain size is measured according to the Japanese Industrial Standard JIS H 0501 (cutting method).

Regulating the preferred dispersion state of the present invention in order to fully demonstrate the effect of obtaining this controlled grain size can be performed by the following two methods.

First, the second-phase particles that exist on the grain boundary should exist at a density of 10⁴ to 10⁸ particles/mm². In this case, it is further preferred that the density be 5 x 10⁵ to 5 x 10⁷ particles/mm².

Second, the value of the ratio r/f of the particle size r (unit: µm) of all of the second-phase particles inside the grain and on the grain boundary and the volume fraction f of the particles should be 1 to 100. The particle size r of the second-phase particles is the arithmetic mean value of the particle size of all of the measured particles. The notation f = 0.005 for the volume fraction f indicates 0.5 vol%.

The inventors discovered that these kinds of second-phase particles possessed the preferred function of improving the stress relaxation resistance. The stress relaxation phenomenon is considered to be caused by dislocations inside the grain moving to the grain boundary, or by grain boundary slippage occurring in part of the grain boundary, with the strain inside the elastic limit changing to permanent strain. In the case of the aforementioned preferred second-phase particles of the present invention, the particles existing inside the grain function to suppress moving of dislocations, and the particles existing at the grain boundary suppress slipping movement of the grain boundary.

Of all these second-phase particles, it is further preferred that the percentage of particles that include Cr as a constituent element be 50% or greater. This is because when Cr is included, the particles can exist as stable compounds without entering the solid solution of Cu even at high temperature. This contributes to a higher density of second-phase particles and increases the effect of suppressing the growth of grain. It is even more preferable that this percentage be 70% or greater. The maximum value of this percentage is not particularly limited, however normally is 90% or less.

By controlling the composition amounts of the main solute components Ni and Si, favorable characteristics can be obtained as follows. The contained amount of Ni is 1.8 to 3.3 mass%, and more preferably 2.0 to 3.0 mass%, and the contained amount of Si is 0.4 to 1.1 mass%, and more preferably 0.5 to 1.0 mass%. Too large of an amount of these elements leads to a drop in electrical conductivity, and causes cracking at the grain boundary by the precipitation at the grain boundary during bending. However, too small of an amount of these elements leads to the insufficient strength.

Cr precipitates as the second-phase particle with Ni or Si, and is effective in controlling the grain size. Furthermore, Cr per se performs precipitation hardening. The contained amount of Cr is 0.01 to 0.5 mass%, and more preferably 0.03 to 0.4 mass%. When the amount is too small, the effect is not obtained, and when the amount is to large, adverse effects occur in that the Cr crystallizes out as coarse crystallized matter during solidification, which causes the plating characteristics to worsen, and promotes starting points for cracking as well as the propagation of cracking during plastic working.

In addition, at least one kind of element that is selected from among (1) at least one of Sn, Mg, Ag, Mn, Ti, Fe and P for a total of 0.01 to 1 mass%, (2) Zn at 0.01 to 10 mass %, and (3) Co at 0.01 to 1.5 mass% can be added in order to improve the alloy characteristics.

These elements improve the strength and the stress relaxation resistance characteristic, and especially Sn and Mg are very effective for that. Zn and Sn function to improve solder joinability, Co functions to improve electrical conductivity, and Mn functions to improve hot workability. When the contained amount when added is too small, the effect is not sufficient, and too large of an amount leads to a drop in electrical conductivity.

In the case of the stress relaxation resistance characteristics, it is preferred that the stress relaxation rate be 30% or less when the material is kept at 165 °C for 3000 hours, and more preferably 25% or less.

The preferred method for manufacturing the copper alloy sheet of the present invention is explained below. The copper alloy sheet of the present invention can, for example, be manufactured by a method comprising the steps of casting, (homogenization) heat treatment, hot working (for example, hot rolling) and cold working (for example, cold rolling) (1), solution heat treatment, cold working (for example, cold rolling) (2), (aging precipitation) heat treatment, cold working (for example cold rolling) (3) and (strain relief) annealing. Here, it is preferred that rapid cooling and facing be performed after heat treatment and before cold working (1).

First, the copper alloy material is prepared by combining all of the elements so that the specified alloy constituent composition is achieved, with the remaining part being Cu and inevitable impurities, and this is melted using a high-frequency melting furnace. Casting is performed at a cooling rate of 0.1 to 100 °C/sec (more preferably, 0.5 to 50 °C/sec) to obtain an ingot. Heat treatment (homogenization) is performed by maintaining the ingot at 900 to 1050 °C for 0.5 to 10 hours (more preferably, for 0.8 to 8 hours). Hot working (hot rolling) is performed at a reduction percentage (rolling reduction) of 50% or greater (more preferably, 60 to 98%), and a processing temperature of 600 °C or greater (more preferably, 620 to 1000 °C) to form a sheet. Rapid cooling (for example, water cooling) is performed by cooling this sheet at a cooling rate of 10 °C/sec or greater (more preferably, 15 to 300 °C/sec). This hot rolled sheet can be faced according to a conventional method. Cold working (cold rolling) (1) is performed with a reduction percentage of 90% or greater (more preferably, 92 to 99%). Solution heat treatment is performed by maintaining the material at 720 to 860 °C for 3 sec to 2 hours (more preferably 5 sec to 0.5 hours). In the solution heat treatment, the treatment is performed within a range of rising temperature from 400 °C to 700 °C and a rate of temperature increase of 0.1 °C/sec to 200 °C/sec (more preferably, 0.5 to 100 °C/sec). Cold working (cold rolling) (2) is performed with a reduction percentage of 5 to 50% (more preferably, 7 to 45%). Aging precipitation heat treatment is performed by maintaining the material at 400 °C to 540 °C for 5 min to 10 hours (more preferably, at 410 to 520 °C for 10 min to 8 hours). Cold working (cold rolling) (3) is performed with a reduction percentage of 10% or less (meaning greater than 0% but not exceeding 10%). Strain relief annealing is performed by maintaining the material at 200 °C to 600 °C for 15 sec to 10 hours (more preferably, 250 to 570 °C for 20 sec to 8 hours).

When there is sufficient strength after aging precipitation heat treatment, cold working (3) and strain relief annealing do not need to be performed after that and can be omitted.

By performing at least one process of the aforementioned processes under the aforementioned conditions and preferable conditions, and particularly by preferably performing all of the processes under the preferable conditions, the specified metallic structure for the copper alloy sheet of the present invention can be obtained. For example, by adjusting the casting speed (cooling speed during casting), it is possible to prevent crystallization of Cr series compounds from occurring excessively. In addition, by adjusting the temperature range and time during which the material is maintained at that temperature during hot rolling, it is possible to suppress coarse precipitation during hot rolling, and suitable precipitation can be performed in a later process. Moreover, the second-phase particles that suppress coarsening of the grain mainly precipitate out during the temperature rise of the solution heat treatment, however, in order to effectively induce that precipitation, it is preferred that processing be performed such that both the processing rate of the cold working (1) process, which is the process prior to the solution heat treatment process, and the rate of temperature rise during the solution heat treatment be within the aforementioned preferred conditions. Furthermore, by employing the cold working (2) process before the aging precipitation heat treatment process, it is possible to induce higher density of microscopic precipitate that contributes to precipitation hardening, and suppress the coarsening of second-phase particles that remain at the time of solutionization during aging precipitation heat treatment.

The copper alloy sheet of the present invention has excellent strength and bending workability, and is suitable for use in electrical / electronic equipment. The preferred copper alloy sheet of this present invention also has excellent electrical conductivity and stress relaxation resistance. With the characteristics described above, the copper alloy sheet of the present invention can also be suitably used in lead frames, connectors, and terminals of electrical / electronic equipment, and is particularly suitable for use in connectors, terminals, relays, switches and sockets that are used in automobiles.

There never before has been material having high strength and high bending workability such as that of the present invention, and this material will improve freedom when designing parts for cutting-edge uses in the future, as well as have a large effect on high functionality of electronic equipment. In addition, by having increased strength makes it possible to make the copper alloy material thinner, thus contributing to a reduction in the amount of global resources used.

### Examples

The present invention will be explained in further detail below based on examples; however, the present invention is not limited to these examples.

### (Examples 1)

An alloy comprising elements that were combined so that their composition was as shown in the table, with the remaining part being Cu and inevitable impurities, was melted in a high-frequency melting furnace, and then cast at a cooling rate of 0.1 to 100 °C/sec to obtain an ingot. After maintaining this ingot at 900 to 1050 °C for 0.5 to 10 hours, a sheet was formed by hot working with the percentage of reduction being 50% or greater and the processing temperature being 600 °C or greater, then the sheet was water cooled at a cooling rate of 10 °C/sec or greater. The hot rolled sheet was then faced, and cold working (1) was performed at a reduction percentage of 90% or greater. Solution heat treatment was then performed by maintaining the sheet at 720 to 860 °C for 3 sec to 2 hours. Solution heat treatment was performed such that the rate of temperature rise during a temperature rise at 400 °C to 700 °C was in the range of 0.1 °C/sec to 200 °C/sec. After that, cold working (2) was performed at a reduction percentage of 5 to 50%, aging precipitation heat treatment was performed by maintaining the material at 400 °C to 540 °C for 5 min to 10 hours, cold working (3) was performed at a reduction percentage of 10% or less, and strain relief annealing was performed by maintaining the material at 200 °C to 600 °C for 15 sec to 10 hours to obtain material to be used as test material. In the case where there was sufficient strength after aging precipitation heat treatment, the cold working (3) and strain relief annealing after that aging precipitation heat treatment were not performed.

The comparative examples given below that are presented with the examples were made outside the range of these manufacturing conditions in order to be separated from the range of examples of the present invention.

Details of the comparative examples are given below.

Comparative example 1-1 is an example in which the cooling rate during the casting process was too low.

Comparative example 1-2 is an example in which the temperature during the homogenization process was too low.

Comparative example 1-3 is an example in which the temperature during the aging precipitation heat treatment process was too high.

Comparative example 1-4 is an example in which the temperature during the homogenization process was too low.

In each of the tables, for example, in the case of the test results of invention example 1-1 as the ID number in Table 1, in regards to the evaluation of the bending workability, judgment results for bending work conditions outside the range of the invention W × T > 0.16 are also displayed on the same line as the judgment results for the bending work conditions within the range of the invention, however, this is done for convenience of listing the ID number. This will be the same for all of the test examples given in each of the tables below.

The characteristics presented below were investigated for these test materials.

### a. Electrical conductivity [EC]

The electrical conductivity (% IACS) was calculated by using the four-terminal method to measure the specific resistance of the material in an isothermal bath that was maintained at 20 °C (±0.5 °C). The spacing between terminals was 100 mm.

### b. Tensile strength [TS]

Three test pieces that were cut out from the direction parallel to the rolling direction according to JIS Z2201-13B were measured according to JIS Z2241, and the average value (MPa) is given.

### c. 180° tight bending workability

Bending work was performed according to JIS Z2248. After preliminary bending was performed using a 0.4 mm R 90° bending die, tight bending was performed using a compression testing machine. The bending location was observed by using a 50x optical microscope to visually inspect whether or not there was cracking on the outside of the bent section. The sheet width W and sheet thickness T conditions of the test piece are indicated in mm. In the table "GW (Good way) " indicates testing in the case where the bending axis is perpendicular to the rolling direction, and "BW (Bad way)" indicates testing in the case where the bending axis is parallel to the rolling direction. In the table, the observation results are indicated as "O (Good)" when no cracking occurred, and as "X (Bad)" when cracking occurred.

### d. Particle size [r], distribution density [p] and volume fraction [f] of the second-phase particles

Observation test pieces were formed by punching the test material into 3 mm diameter pieces, and polishing the pieces to a thin film by using a twin-jet polishing method. Using a transmission electron microscope having an accelerating voltage of 300 kV, 5000x photographs were taken arbitrarily every ten fields of view, and the particle size r (µm) and distribution density ρ (particles/mm²) were measured on the photographs. The particle size r of the second-phase particles was found by first, finding the particle size of each particle, then, for all of the measured particles, finding the calculated average value of the particle sizes of all of the particles. The particle size of each particle was taken to be the calculated average value of the long diameter and short diameter of the particle. Moreover, the thickness of an observed test piece was measured from the thickness contours, and of the total volume of an observed field of view, the percentage of the volume occupied by the second-phase particles was taken to be the volume fraction f.

### e. Identification of second-phase constituent atoms [C]

An EDX spectrometer that was attached to the TEM was used. Analysis was performed for 20 second-phase particles, and the percentage of the total number measured comprising Cr was calculated.

### f. Stress relaxation resistance [SR]

The stress relaxation resistance was measured according to the Japan Electronics and Information Technology Industries Association standards EMAS-3003 under conditions of 165 °C for 3000 hours. An initial stress that was 80% the offset yield strength (proof stress) was applied by the cantilever method.

FIG. 1 is a drawing explaining the method for testing the stress relaxation, where (a) of FIG. 1 shows the state before heat treatment, and (b) of FIG. 1 shows the state after heat treatment. The stress relaxation rate (%) was calculated as (Ht - H₁)/δ₀ × 100.

### g. Average grain size [GS]

The average grain size was measured according to JIS H 0501 (cutting method). Measurement was performed for a cross-section that is parallel to the rolling direction, and a cross-section that is perpendicular to the rolling direction, and the average of both was taken. Observation of the metallic structure was done by chemically edging a mirror polished material surface and performing SEM reflection electron imaging.

[Table 1]

**TABLE 1**

| ID Number | Alloy composition | | | *ρ* | *T* | Bending workability (Cracking Y/N) (W unit: mm) | | | | | | TS | % of particles comprising Cr | GS | EC | SR |
|---|---|---|---|---|---|---|---|---|---|---|---|---|---|---|---|---|
| | Ni | Si | Cr | | | GW | | | BW | | | | | | | |
| | mass% | mass% | mass% | Particles/mm² | mm | W=0.5 | W=1 | W=2 | W=0.5 | W=1 | W=2 | MPa | % | *µ*m | %IACS | % |
| Invention example 1-1 | 1.81 | 0.50 | - | 6 × 10⁴ | 0.30 | ○ | × | × | ○ | × | × | 742 | 0 | 5.2 | 42.1 | 28.2 |
| Invention example 1-2 | 2.32 | 0.65 | - | 9 × 10⁴ | 0.25 | ○ | × | × | ○ | × | × | 770 | 0 | 4.3 | 40.2 | 27.4 |
| Invention example 1-3 | 2.81 | 0.79 | - | 7 × 10⁵ | 0.20 | ○ | × | × | ○ | × | × | 784 | 0 | 6.8 | 39.5 | 28.1 |
| Invention example 1-4 | 3.28 | 0.94 | - | 2 × 10⁶ | 0.15 | ○ | ○ | × | ○ | ○ | × | 792 | 0 | 7.0 | 38.6 | 26.7 |
| Invention example 1-5 | 1.83 | 0.50 | 0.21 | 2 × 10⁵ | 0.08 | ○ | ○ | ○ | ○ | ○ | ○ | 755 | 85 | 4.8 | 43.2 | 28.6 |
| Invention example 1-6 | 2.36 | 0.65 | 0.15 | 3 × 10⁸ | 0.15 | ○ | ○ | × | ○ | ○ | × | 769 | 75 | 5.5 | 39.5 | 28.3 |
| Invention example 1-7 | 2.84 | 0.79 | 0.11 | 2 × 10⁷ | 0.12 | ○ | ○ | × | ○ | ○ | × | 785 | 95 | 4.2 | 38.2 | 27.5 |
| Invention example 1-8 | 3.24 | 0.94 | 0.25 | 8 × 10⁷ | 0.08 | ○ | ○ | ○ | ○ | ○ | ○ | 805 | 90 | 6.2 | 36.1 | 26.8 |
| Comparative example 1-1 | 2.34 | 0.66 | - | 3 × 10³ | 0.25 | × | × | × | × | × | × | 725 | 0 | 13.5 | 39.2 | 28.2 |
| Comparative example 1-2 | 2.82 | 0.77 | - | 7 × 10³ | 0.20 | × | × | × | × | × | × | 762 | 0 | 18.2 | 38.2 | 29.3 |
| Comparative example 1-3 | 2.35 | 0.62 | 0.15 | 2 × 19⁹ | 0.30 | × | × | × | × | × | × | 719 | 65 | 12.9 | 39.5 | 28.0 |
| Comparative example 1-4 | 2.81 | 0.75 | 0.21 | 5 × 10³ | 0.15 | × | × | × | × | × | × | 758 | 45 | 17.5 | 37.5 | 27.9 |

| | | | | | | | | | | | | | | | | |
|---|---|---|---|---|---|---|---|---|---|---|---|---|---|---|---|---|
| × -not belonging to the present invention | | | | | | | | | | | | | | | | |

As can be clearly seen from Table 1, invention examples 1-1 to 1-8 have excellent strength, electrical conductivity, bending workability and stress relaxation resistance characteristics. However, when some of the elements of the present invention are not satisfied, some characteristics may become inferior. For example, comparative examples 1-1 to 1-4 are all examples in which the bending workability is inferior. In comparative examples 1-1, 1-2 and 1-4, the density of precipitate on the grain boundary is low, and the grain size becomes coarse. Moreover, in comparative example 1-3, the density of precipitate on the grain boundary is high, and it was observed that cracking occurred at the grain boundary.

### (Examples 2)

The same investigation as was performed for examples 1 was performed for a copper alloy comprising the composition shown in Table 2 with the remaining part being Cu and inevitable impurities. The manufacturing method and measurement method were the same as for examples 1.

The comparative examples given below that are presented with the examples were made outside the range of these manufacturing conditions in order to be separated from the range of examples of the present invention. Details of the comparative examples are given below.

Comparative example 2-1 is an example in which the processing rate during cold working (cold rolling) was too low.

Comparative example 2-2 is an example in which the temperature during the homogenization process was too low.

Comparative example 2-3 is an example in which the cooling rate during the casting process was too low.

Comparative example 2-4 is an example in which the temperature during the homogenization process was too low.

[Table 2]

**TABLE 2**

| ID Number | Alloy composition | | | r/f | T | Bending workability (Cracking Y/N) (W unit: mm) | | | | | | TS | % of particles comprising Cr | GS | EC | SR |
|---|---|---|---|---|---|---|---|---|---|---|---|---|---|---|---|---|
| | Ni | Si | Cr | | | GW | | | BW | | | | | | | |
| | mass% | mass% | mass% | | mm | W=0.5 | W=1 | W=2 | W=0.5 | W=1 | W=2 | MPa | % | *µ*m | %IACS | % |
| Invention example 2-1 | 1.91 | 0.55 | - | 45.1 | 0.30 | ○ | × | × | ○ | × | × | 743 | 0 | 7.1 | 41.8 | 27.1 |
| Invention example 2-2 | 2.41 | 0.68 | - | 15.4 | 0.25 | ○ | × | × | ○ | × | × | 772 | 0 | 5.8 | 40.6 | 26.7 |
| Invention example 2-3 | 2.72 | 0.75 | - | 17.2 | 0.20 | ○ | × | × | ○ | × | × | 789 | 0 | 6.2 | 39.8 | 28.2 |
| Invention example 2-4 | 3.11 | 0.89 | - | 10.4 | 0.15 | ○ | ○ | × | ○ | ○ | × | 790 | 0 | 4.7 | 38.2 | 27.6 |
| Invention example 2-5 | 1.93 | 0.55 | 0.21 | 25.2 | 0.25 | ○ | × | × | ○ | × | × | 751 | 90 | 5.6 | 43.1 | 26.3 |
| Invention example 2-6 | 2.45 | 0.68 | 0.15 | 12.1 | 0.15 | ○ | ○ | × | ○ | ○ | × | 773 | 80 | 6.3 | 39.6 | 28.5 |
| Invention example 2-7 | 2.76 | 0.75 | 0.11 | 5.4 | 0.10 | ○ | ○ | × | ○ | × | × | 783 | 85 | 4.5 | 38.3 | 27.4 |
| Invention example 2-8 | 3.18 | 0.89 | 0..25 | 72.3 | 0.08 | ○ | ○ | ○ | ○ | ○ | ○ | 802 | 75 | 7.4 | 36.6 | 26.8 |
| Comparative example 2-1 | 2.44 | 0.66 | - | 24.5 | 0.15 | ○ | × | × | ○ | × | × | 680 | 0 | 5.2 | 42.1 | 29.5 |
| Comparative example 2-2 | 2.74 | 0.76 | - | 145.7 | 0.30 | × | × | × | × | × | × | 771 | 0 | 19.3 | 39.5 | 30.2 |
| Comparative example 2-3 | 2.41 | 0.65 | 0.15 | 0.71 | 0.12 | × | × | × | × | × | × | 765 | 45 | 18.2 | 39.1 | 29.2 |
| Comparative example 2-4 | 2.72 | 0.73 | 0.15 | 120.2 | 0.25 | × | × | × | × | × | × | 761 | 75 | 16.2 | 37.5 | 27.8 |

| | | | | | | | | | | | | | | | | |
|---|---|---|---|---|---|---|---|---|---|---|---|---|---|---|---|---|
| × - not belonging to the present invention | | | | | | | | | | | | | | | | |

As can be clearly seen from Table 2, invention examples 2-1 to 2-8 have excellent strength, electrical conductivity, bending workability and stress relaxation resistance characteristics. However, when some of the elements of the present invention are not satisfied, some characteristics may become inferior. For example, comparative example 2-1 is an example in which the tensile strength became inferior. In this comparative example 2-1, the solutionization temperature was lowered and grain size was made small, however, precipitation hardening was thought to be insufficient and there was not enough strength. Comparative examples 2-2 and 2-4 are examples in which the bending workability became inferior. In these comparative examples 2-2 and 2-4, it was found that the precipitation fraction was small, so the r/f value became large and the grain size became coarse. Comparative example 2-3 is an example in which bending workability was inferior. In this comparative example 2-3, it was found that the size of the second-phase particles was small, so the r/f value became small, and because the grain could not be effectively controlled, the grain size became coarse.

### (Examples 3)

The same investigation as was performed for examples 1 was performed for a copper alloy comprising the composition shown in Table 3 with the remaining part being Cu and inevitable impurities. The manufacturing method and measurement method were the same as for examples 1.

The comparative examples below that are presented with the examples in Table 3 were made with the contained amounts of Ni and Si outside the preferred range of the present invention.

[Table 3]

**TABLE 3**

| ID Number | Alloy composition | | | Other added elements | *ρ* | T | Bending workability (Cracking Y/N) (W unit mm) | | | | | | TS | % of particles comprising Cr | GS | EC | SR |
|---|---|---|---|---|---|---|---|---|---|---|---|---|---|---|---|---|---|
| | Ni | Si | Cr | | | | GW | | | BW | | | | | | | |
| | mass% | mass% | mass% | mass% | Particles/mm² | mm | W=0.5 | W=1 | W=2 | W=0.5 | W=1 | W=2 | MPa | % | *µ*m | %IACS | % |
| Invention example 3-1 | 1.81 | 0.51 | 0.15 | 0.1Mn, 0.05P | 6 × 10⁴ | 0.20 | ○ | × | × | ○ | × | × | 748 | 85 | 5.2 | 38.2 | 26.2 |
| Invention example 3-2 | 2.31 | 0.65 | 0.18 | 0.1Mg, 0.15Sn, 0.5Zn | 9 × 10⁴ | 0.25 | ○ | × | × | ○ | × | × | 765 | 75 | 4.8 | 39.1 | 23.6 |
| Invention example 3-3 | 2.81 | 0.77 | 0.21 | 0.3Ag, 0.1Ti | 8 × 10⁵ | 0.15 | ○ | ○ | × | ○ | ○ | × | 772 | 80 | 6.2 | 37.2 | 27.3 |
| Invention example 3-4 | 3.26 | 0.92 | 0.19 | 0.2Co, 0.1Fe | 7 × 10⁵ | 0.10 | ○ | ○ | × | ○ | ○ | × | 790 | 90 | 7.1 | 37.2 | 26.1 |
| Comparative example 3-1 | 1.61 | 0.31 | 0.15 | 0.2Sn, 0.1 5Mg | 6 × 10⁵ | 0.20 | ○ | × | × | ○ | × | × | 710 | 85 | 8.2 | 41.2 | 31.2 |
| Comparative example 3-2 | 3.51 | 1.21 | 0.12 | 0.3Mn | 2 × 10⁵ | 0.15 | ○ | × | × | ○ | × | × | 795 | 85 | 8.9 | 32.5 | 26.0 |

| | | | | | | | | | | | | | | | | | |
|---|---|---|---|---|---|---|---|---|---|---|---|---|---|---|---|---|---|
| × - not belonging to the present invention | | | | | | | | | | | | | | | | | |

As can be clearly seen from Table 3, invention examples 3-1 to 3-4, in which the contained amounts of Ni and Si are especially within the preferred range, have excellent strength, electrical conductivity, bending workability, and stress relaxation resistance characteristics. However, when the added amounts of Ni and Si are not especially within the preferred range, some characteristics may become inferior. For example, comparative example 3-1 is an example in which the amounts of Ni and Si were inadequate, so there was insufficient strength. Comparative example 3-2 is an example in which the amounts of Ni and Si were large, so precipitation occurred at the grain boundary, causing the bending workability to become somewhat inferior. Of course it is not necessary for the contained amounts of Ni and Si to be especially within the preferred range, however, when outside this range, examples are seen in which characteristics become inferior, so it is preferred that when possible, the amount of Ni be within the range 1.8 to 3.3 mass%, and that the amount of Si be within the range 0.4 to 1.1 mass%.

### (Examples 4)

The same investigation as was performed for examples 1 was performed for a copper alloy comprising the composition shown in Table 4 with the remaining part being Cu and inevitable impurities. The manufacturing method and measurement method were the same as for examples 1.

The comparative examples below that are presented with the examples in Table 4 were made with the contained amounts of other added elements outside the preferred range of the present invention.

[Table 4]

**TABLE 4**

| ID Number | Alloy composition | | | Other added elements | r/f | T | Bending workability (Cracking Y/N) (W unit mm) | | | | | | TS | % of particles comprising Cr | GS | EC | SR |
|---|---|---|---|---|---|---|---|---|---|---|---|---|---|---|---|---|---|
| | Ni | Si | Cr | | | | GW | | | BW | | | | | | | |
| | mass% | mass% | mass% | mass% | | mm | W=0.5 | W=1 | W=2 | W=0.5 | W=1 | W=2 | MPa | % | *µ*m | %IACS | % |
| Invention example 4-1 | 1.91 | 0.57 | 0.15 | 0.2Co, 0.2Mn | 23.2 | 0.20 | ○ | × | × | ○ | × | × | 751 | 70 | 6.8 | 38.3 | 27.2 |
| Invention example 4-2 | 2.42 | 0.60 | 0.22 | 0.2Fe, 0.03P | 44.2 | 0.15 | ○ | ○ | × | ○ | × | × | 765 | 75 | 7.8 | 39.6 | 27.8 |
| Invention example 4-3 | 2.74 | 0.71 | 0.1 | 0.2Ag. 0.3Ti | 35.2 | 0.12 | ○ | ○ | × | ○ | ○ | × | 780 | 80 | 7.2 | 37.6 | 25.6 |
| Invention example 4-4 | 3.18 | 0.60 | 0.2 | 0.4Sn, 1.0Zn, 0.1Mg | 7.8 | 0.08 | ○ | ○ | ○ | ○ | ○ | ○ | 802 | 85 | 5.1 | 38.0 | 24.2 |
| Comparative example 4-1 | 2.46 | 0.62 | 0.15 | 1.2Sn, 1.2Mg | 125.4 | 0.15 | ○ | × | × | × | × | × | 785 | 40 | 12.2 | 28.0 | 33.2 |
| Comparative example 4-2 | 2.77 | 0.70 | 0.17 | 1.5Fe | 144.2 | 0.12 | ○ | ○ | ○ | ○ | ○ | ○ | 669 | 35 | 13.1 | 25.2 | 40.2 |

| | | | | | | | | | | | | | | | | | |
|---|---|---|---|---|---|---|---|---|---|---|---|---|---|---|---|---|---|
| × - not belonging to the present invention | | | | | | | | | | | | | | | | | |

As is clearly shown in Table 4, invention examples 4-1 to 4-4, in which the contained amounts of other added elements (secondary added elements) other than Ni and Si were especially within the preferred range, have excellent electrical conductivity, bending workability and stress relaxation resistance characteristics. However, when the contained amounts of those other added elements are not especially within the preferred range, some of the characteristics may become inferior. For example, comparative example 4-1 is an example in which the bending workability became inferior. In this comparative example 4-1, it is thought that because the contained amount of the secondary added elements was too large, the grain boundary became fragile. Comparative example 4-2 is an example in which the mechanical strength became inferior. In this comparative example 4-2, it is thought that because the contained amount of the secondary added elements was too large, compounds other than Ni-Si series compounds that contribute to precipitation hardening were formed. Of course, it is not necessary that the contained amounts of secondary added elements be especially within the preferred range, however, by being outside of this range, examples were seen in which characteristics become inferior, so when adding other added elements, it is preferred when possible that one or two or more kinds of elements be included from among at least one of Sn, Mg, Ag, Mn, Ti, Fe and P at a total of 0.01 to 1 mass%, Zn at 0.01 to 10 mass%, and Co at 0.01 to 1.5 mass%.

The results of examples 1 to 4 above are shown in FIG. 2. It can be seen that with the examples of the invention, under the conditions of 180° tight bending and material dimensions where the product of the test piece thickness T and the test piece width W is 0.16 or less, processing was possible with no cracking; however, for the comparative examples, processing was not possible.

### Industrial Applicability

The copper alloy sheet of the present invention can be suitably applied for use in lead frames, connectors and terminal materials for electrical / electronic equipment, for example, connectors, terminal materials, relays, switches and sockets for use in automobiles.

## Claims

1. A copper alloy sheet having a tensile strength of 730 to 820 MPa, and consisting of:
1.8 to 3.3 mass% of Ni,
0.4 to 1.1 mass% of Si,
0.01 to 0.5 mass% of Cr,
optionally 0.01 to 1 mass% in total of at least one element selected from Sn, Mg, Ag, Mn, Ti, Fe and P,
optionally 0.01 to 1.0 mass% of Zn, and
optionally 0.01 to 1.5 mass% of Co,
with the balance being Cu and inevitable impurities;
wherein when the sheet width and the sheet thickness at the time where the copper alloy sheet is bent by 180° tight bending, the bending work being performed according to JIS Z2248, without causing any cracks are taken to be W, in a unit of mm, and T, in a unit of mm, the product of W and T, in a unit of mm², is 0.16 or less;
wherein second-phase particles existing on a grain boundary exist at a density of 10⁴ to 10⁸ particles/mm², and the average grain size is 10 µm or less; and
wherein the copper alloy sheet is obtainable by a method comprising the steps of:
casting at a cooling rate of 0.1 to 100°C/sec;
heat treatment or homogenization heat treatment at 900 to 1050°C for 0.5 to 10 hours;
hot working at a reduction percentage of 50% or greater, and a processing temperature of 600°C or greater, followed by rapid cooling at a cooling rate of 10°C/sec or greater;
cold working (1) with a reduction percentage of 90% or greater;
solution heat treatment at 720 to 860°C for 3 sec to 2 hours, wherein during the rise of temperature from 400°C to 700°C, a rate of temperature rise is 0.1°C/sec to 200°C/sec;
cold working (2) with a reduction percentage of 5 to 50%;
heat treatment or aging precipitation heat treatment at 400°C to 540°C for 5 min to 10 hours,
cold working (3) with a reduction percentage of greater than 0% but not exceeding 10%, and
annealing or strain relief annealing at 200°C to 600°C for 15 sec to 10 hours.

2. A copper alloy sheet having a tensile strength of 730 to 820 MPa, and consisting of:
1.8 to 3.3 mass% of Ni,
0.4 to 1.1 mass% of Si,
0.01 to 0.5 mass% of Cr,
optionally 0.01 to 1 mass% in total of at least one element selected from Sn, Mg, Ag, Mn, Ti, Fe and P,
optionally 0.01 to 1.0 mass% of Zn, and
optionally 0.01 to 1.5 mass% of Co,
with the balance being Cu and inevitable impurities;
wherein when the sheet width and the sheet thickness at the time where the copper alloy sheet is bent by 180° tight bending, the bending work being performed according to JIS Z2248, without causing any cracks are taken to be W, in a unit of mm, and T, in a unit of mm, the product of W and T, in a unit of mm², is 0.16 or less;
wherein the value of ratio r/f of the particle size r, in a unit of µm, of second-phase particles inside the grain and on the grain boundary and the volume fraction f, in a unit of vol.%, of the particles is at least 1 and not more than 100 µm/vol.%, and the average grain size is 10 µm or less; and wherein the copper alloy sheet is obtainable by a method comprising the steps of:
casting at a cooling rate of 0.1 to 100°C/sec;
heat treatment or homogenization heat treatment at 900 to 1050°C for 0.5 to 10 hours;
hot working at a reduction percentage of 50% or greater, and a processing temperature of 600°C or greater, followed by rapid cooling at a cooling rate of 10°C/sec or greater;
cold working (1) with a reduction percentage of 90% or greater;
solution heat treatment at 720 to 860°C for 3 sec to 2 hours, wherein during the rise of temperature from 400°C to 700°C, a rate of temperature rise is 0.1°C/sec to 200°C/sec;
cold working (2) with a reduction percentage of 5 to 50%;
heat treatment or aging precipitation heat treatment at 400°C to 540°C for 5 min to 10 hours,
cold working (3) with a reduction percentage of greater than 0% but not exceeding 10%, and
annealing or strain relief annealing at 200°C to 600°C for 15 sec to 10 hours.

3. The copper alloy sheet of claim 1 or claim 2, wherein of said second-phase particles, the ratio of particles comprising Cr as a constituent element is 50% or more.

4. The copper alloy sheet of any one of the claims 1 to 3, wherein, when the copper alloy sheet is maintained at 165 °C for 3000 hours, the stress relaxation rate is 30% or less.

## Patentansprüche

1. Kupferlegierungsblech, das eine Zugfestigkeit von 730 bis 820 MPa aufweist, und bestehend aus:
1,8 bis 3,3 Massen-% Ni,
0,4 bis 1,1 Massen-% Si,
0,01 bis 0,5 Massen-% Cr,
optional insgesamt 0,01 bis 1 Massen-% von mindestens einem Element, das aus Sn, Mg, Ag, Mn, Ti, Fe und P ausgewählt wird,
optional 0,01 bis 1,0 Massen-% Zn, und
optional 0,01 bis 1,5 Massen-% Co,
wobei der Ausgleich Kupfer und unvermeidliche Verunreinigungen sind;
wobei, wenn die Blechbreite und die Blechdicke zum Zeitpunkt, in dem das Kupferlegierungsblech durch enges Biegen um 180° gebogen wird, wobei die Biegetätigkeit gemäß JIS Z2248 durchgeführt wird, ohne dass irgendwelche Risse verursacht werden, als W, in einer Einheit von mm, und T, in einer Einheit von mm, angenommen werden, das Produkt von W und T, in einer Einheit von mm², 0,16 oder weniger beträgt;
wobei Partikel einer zweiten Phase auf einem Kornrand mit einer Dichte von 10⁴ bis 10⁸ Partikel/mm² vorhanden sind, und wobei die durchschnittliche Korngröße 10 µm oder weniger beträgt; und
wobei das Kupferlegierungsblech durch ein Verfahren erhältlich ist, das die folgenden Schritte umfasst:
Gießen mit einer Kühlgeschwindigkeit von 0,1 bis 100°C/Sekunde;
Wärmebehandlung oder Homogenisierungswärmebehandlung bei 900 bis 1050°C für 0,5 bis 10 Stunden;
warmes Bearbeiten mit einem Reduktionsprozentanteil von 50% oder größer, und einer Verarbeitungstemperatur von 600°C oder größer, gefolgt von schnellem Abkühlen mit einer Abkühlgeschwindigkeit von 10°C/Sekunde oder größer;
kaltes Bearbeiten (1) mit einem Reduktionsprozentanteil von 90% oder größer;
Lösungswärmebehandlung bei 720 bis 860°C für 3 Sekunden bis 2 Stunden, wobei während des Anstiegs der Temperatur von 400°C bis 700°C eine Geschwindigkeit des Temperaturanstiegs 0,1°C/Sekunde bis 200°C/Sekunde beträgt;
kaltes Bearbeiten (2) mit einem Reduktionsprozentanteil von 5 bis 50%;
Wärmebehandlung oder Alterungsausscheidungswärmebehandlung bei 400°C bis 540°C für 5 Minuten bis 10 Stunden,
kaltes Bearbeiten (3) mit einem Reduktionsprozentanteil von größer als 0%, aber 10% nicht überschreitend, und
Ausglühen oder Ausglühen zur Spannungsentlastung bei 200°C bis 600°C für 15 Sekunden bis 10 Stunden.

2. Kupferlegierungsblech, das eine Zugfestigkeit von 730 bis 820 MPa aufweist, und bestehend aus:
1,8 bis 3,3 Massen-% Ni,
0,4 bis 1,1 Massen-% Si,
0,01 bis 0,5 Massen-% Cr,
optional insgesamt 0,01 bis 1 Massen-% von mindestens einem Element, das aus Sn, Mg, Ag, Mn, Ti, Fe und P ausgewählt wird,
optional 0,01 bis 1,0 Massen-% Zn, und
optional 0,01 bis 1,5 Massen-% Co,
wobei der Ausgleich Kupfer und unvermeidliche Verunreinigungen sind;
wobei, wenn die Blechbreite und die Blechdicke zum Zeitpunkt, in dem das Kupferlegierungsblech durch enges Biegen um 180° gebogen wird, wobei die Biegetätigkeit gemäß JIS Z2248 durchgeführt wird, ohne dass irgendwelche Risse verursacht werden, als W, in einer Einheit von mm, und T, in einer Einheit von mm, angenommen werden, das Produkt von W und T, in einer Einheit von mm², 0,16 oder weniger beträgt;
wobei der Wert des Verhältnisses r/f der Partikelgröße r, in einer Einheit von µm, von Partikeln einer zweiten Phase innerhalb des Korns und auf dem Kornrand und des Volumenanteils f, in einer Einheit von Volumen-%, der Partikel mindestens 1 und nicht mehr als 100 µm/Volumen-% beträgt, und die durchschnittliche Korngröße 10 µm oder weniger beträgt; und
wobei das Kupferlegierungsblech durch ein Verfahren erhältlich ist, das die folgenden Schritte umfasst:
Gießen mit einer Kühlgeschwindigkeit von 0,1 bis 100°C/Sekunde;
Wärmebehandlung oder Homogenisierungswärmebehandlung bei 900 bis 1050°C für 0,5 bis 10 Stunden;
warmes Bearbeiten mit einem Reduktionsprozentanteil von 50% oder größer, und einer Verarbeitungstemperatur von 600°C oder größer, gefolgt von schnellem Abkühlen mit einer Abkühlgeschwindigkeit von 10°C/Sekunde oder größer;
kaltes Bearbeiten (1) mit einem Reduktionsprozentanteil von 90% oder größer;
Lösungswärmebehandlung bei 720 bis 860°C für 3 Sekunden bis 2 Stunden, wobei während des Anstiegs der Temperatur von 400°C bis 700°C eine Geschwindigkeit des Temperaturanstiegs 0,1°C/Sekunde bis 200°C/Sekunde beträgt;
kaltes Bearbeiten (2) mit einem Reduktionsprozentanteil von 5 bis 50%;
Wärmebehandlung oder Alterungsausscheidungswärmebehandlung bei 400°C bis 540°C für 5 Minuten bis 10 Stunden,
kaltes Bearbeiten (3) mit einem Reduktionsprozentanteil von größer als 0%, aber 10% nicht überschreitend, und
Ausglühen oder Ausglühen zur Spannungsentlastung bei 200°C bis 600°C für 15 Sekunden bis 10 Stunden.

3. Kupferlegierungsblech nach Anspruch 1 oder Anspruch 2, wobei bei den Partikeln der zweiten Phase das Verhältnis der Partikel, die Cr als ein Bestandteilselement umfassen, 50% oder mehr beträgt.

4. Kupferlegierungsblech nach einem beliebigen der Ansprüche 1 bis 3, wobei, wenn das Kupferlegierungsblech bei 165°C für 3000 Stunden gehalten wird, die Spannungsrelaxationsrate 30% oder weniger beträgt.

## Revendications

1. Feuille d'alliage de cuivre ayant une résistance à la traction allant de 730 à 820 MPa, et constituée de :
1,8 à 3,3% en masse de Ni,
0,4 à 1,1% en masse de Si,
0,01 à 0,5% en masse de Cr,
éventuellement 0,01 à 1% en masse au total d'au moins un élément choisi parmi Sn, Mg, Ag, Mn, Ti, Fe et P,
éventuellement 0,01 à 1,0% en masse de Zn, et
éventuellement 0,01 à 1,5% en masse de Co,
le reste étant du Cu et des impuretés inévitables ;
où lorsque la largeur de la feuille et l'épaisseur de la feuille au moment où la feuille d'alliage de cuivre est pliée par un pliage serré à 180°, le travail de pliage étant effectué conformément à la Norme JIS Z2248, sans provoquer des fissures sont désignées par W, en unité mm, et T, en unité mm, le produit de W et T, en unité mm², est inférieur ou égal à 0,16 ;
où des particules de phase secondaire existant sur un joint de grain, existent à une densité allant de 10⁴ à 10⁸ particules/mm², et la taille moyenne de grain est inférieure ou égale à 10 µm ; et
où la feuille d'alliage de cuivre peut être obtenue par un procédé comprenant les étapes suivantes :
la coulée à une vitesse de refroidissement allant de 0,1 à 100°C/s ;
un traitement thermique ou un traitement thermique d'homogénéisation à une température allant de 900 à 1050°C pendant 0,5 à 10 heures ;
le travail à chaud à un pourcentage de réduction supérieur ou égal à 50%, et à une température de traitement supérieure ou égale à 600°C, suivi d'un refroidissement rapide à une vitesse de refroidissement supérieure ou égale à 10°C/s ;
le travail à froid (1) avec un pourcentage de réduction supérieur ou égal à 90% ;
un traitement thermique de mise en solution à une température allant de 720 à 860°C pendant 3 secondes à 2 heures, où, au cours de l'élévation de température de 400°C à 700°C, une vitesse d'élévation de température est de 0,1°C/s à 200°C/s ;
le travail à froid (2) avec un pourcentage de réduction allant de 5 à 50% ;
un traitement thermique ou un traitement thermique de précipitation par vieillissement à une température allant de 400°C à 540°C pendant 5 minutes à 10 heures,
le travail à froid (3) avec un pourcentage de réduction supérieur à 0% mais ne dépassant pas 10%, et
le recuit ou le recuit de détente des contraintes à une température allant de 200°C à 600°C pendant 15 secondes à 10 heures.

2. Feuille d'alliage de cuivre ayant une résistance à la traction allant de 730 à 820 MPa, et constituée de :
1,8 à 3,3% en masse de Ni,
0,4 à 1,1% en masse de Si,
0,01 à 0,5% en masse de Cr,
éventuellement 0,01 à 1% en masse au total d'au moins un élément choisi parmi Sn, Mg, Ag, Mn, Ti, Fe et P,
éventuellement 0,01 à 1,0% en masse de Zn, et
éventuellement 0,01 à 1,5% en masse de Co,
le reste étant du Cu et des impuretés inévitables ;
où lorsque la largeur de la feuille et l'épaisseur de la feuille au moment où la feuille d'alliage de cuivre est pliée par un pliage serré à 180°, le travail de pliage étant effectué conformément à la Norme JIS Z2248, sans provoquer des fissures sont désignées par W, en unité mm, et T, en unité mm, le produit de W et T, en unité mm², est inférieur ou égal à 0,16 ;
où la valeur du rapport r/f de la taille de particule r, en unité µm, des particules de phase secondaire à l'intérieur du grain et sur le joint de grain et de la fraction volumique f, en unité % en volume, des particules est supérieure ou égale à 1 et inférieure ou égale 100 µm/% en volume, et la taille moyenne de grain est inférieure ou égale à 10 µm ; et où la feuille d'alliage de cuivre peut être obtenue par un procédé comprenant les étapes suivantes :
la coulée à une vitesse de refroidissement allant de 0,1 à 100°C/s ;
un traitement thermique ou un traitement thermique d'homogénéisation à une température allant de 900 à 1050°C pendant 0,5 à 10 heures ;
le travail à chaud à un pourcentage de réduction supérieur ou égal à 50%, et à une température de traitement supérieure ou égale à 600°C, suivi d'un refroidissement rapide à une vitesse de refroidissement supérieure ou égale à 10°C/s ;
le travail à froid (1) avec un pourcentage de réduction supérieur ou égal à 90% ;
le traitement thermique de mise en solution à une température allant de 720 à 860°C pendant 3 secondes à 2 heures, où, au cours de l'élévation de température de 400°C à 700°C, une vitesse d'élévation de température est de 0,1°C/s à 200°C/s,
le travail à froid (2) avec un pourcentage de réduction allant de 5 à 50% ;
un traitement thermique ou un traitement thermique de précipitation par vieillissement à une température allant de 400°C à 540°C pendant 5 minutes à 10 heures,
le travail à froid (3) avec un pourcentage de réduction supérieur à 0% mais ne dépassant pas 10%, et
le recuit ou le recuit de détente des contraintes à une température allant de 200°C à 600°C pendant 15 secondes à 10 heures.

3. Feuille d'alliage de cuivre de la revendication 1 ou 2, dans laquelle, le rapport de particules, desdites particules de phase secondaire, comprenant du Cr en tant qu'élément constitutif est supérieur ou égal à 50%.

4. Feuille d'alliage de cuivre de l'une quelconque des revendications 1 à 3, dans laquelle, lorsque la feuille d'alliage de cuivre est maintenue à 165°C pendant 3000 heures, le taux de relaxation des contraintes est inférieur ou égal à 30%.
